

Sept. 19, 1944.

N. H. STEWART

2,358,668

X-RAY TUBE ANODE SEAL

Filed Jan. 27, 1942

*Fig. 1.*



*Fig. 2.*



*Fig. 3.*



*Fig. 4.*



INVENTOR  
N. H. STEWART.

BY  
John Greenhaw  
ATTORNEY

## UNITED STATES PATENT OFFICE

2,358,668

## X-RAY TUBE ANODE SEAL

Nelson H. Stewart, Caldwell, N. J., assignor to Westinghouse Electric & Manufacturing Company, East Pittsburgh, Pa., a corporation of Pennsylvania

Application January 27, 1942, Serial No. 428,358

3 Claims. (Cl. 250—149)

This invention relates to the fabrication of an anode for an X-ray tube, especially to such anodes which include a copper rod supporting a press element of the alloy known as "Kovar" or like metal capable of being readily united to the glass of the press, and the invention relates more particularly to the joint between the copper rod and the "Kovar" and the method of forming such union.

In the usual type of copper anode using a Kovar seal, the Kovar is soldered to the anode after the anode has been machined. In addition to the fact that some losses are experienced due to poor soldering, the latter constitutes an extra operation which can be avoided, thus cheapening the manufacturing costs of an anode, according to the results attending my researches in this field.

Accordingly, an object of this invention is to avoid the disadvantages and inconveniences incidental to the use of a soldered joint between the Kovar element and its copper support by eliminating the use of solder in that connection.

Another object is to cut down the number of operations in forming the aforesaid joint by uniting the Kovar to the copper at the same time that the copper is cast.

A further object is to provide means to produce the cast Kovar-copper joint in such a manner that the cast product can be readily machined to a shape which facilitates the step of sealing the Kovar element into the glass press by which the anode is eventually integrated with the X-ray tube.

Still another object is to provide apparatus which can be used over and over for the fabrication, seriatim, in quantity production, of anodes made according to the present invention, each of the anodes constituting a complete anode unit as an intermediate product ready for incorporation in its X-ray tube by the use of substantially conventional machinery.

A cognate object is to provide a complete anode unit of relatively few, sturdy parts, free from the presence of residual corrosive material used in every soldered joint, in place of which is utilized, according to my invention, a thoroughly reliable cast union between the copper supporting rod and the Kovar seal, the novel anodes thus produced being capable of being stored, transported and supplied in desired quantities as such.

Other objects and features of the invention will be made apparent to those skilled in the art as progress is made with the description of the embodiment of the invention selected for illustration in the accompanying drawing wherein:

Fig. 1 is a view in side elevation, partly in section, of an anode for an X-ray tube, in the construction of which the present invention has been embodied;

5 Fig. 2 is a view in vertical section, showing an assembly of the component elements for making the anode of Fig. 1 and including the crucible in which said assembly is placed ready for subjection to the heat of a suitable furnace;

10 Fig. 3 is a view in sectional elevation illustrating the assembly of Fig. 2 disposed within the furnace, and showing the parts in their position after application of the necessary heat;

15 Fig. 4 shows the anode removed from the furnace and crucible and partly machined.

Referring now to the drawing in detail, the part designated by the reference character 11 is a copper rod which in the instance shown is to constitute the body of the anode in the completed product, the latter being shown in Fig. 1, while in Fig. 2 the copper element is indicated as a slug at 10, being as yet unshaped.

20 A crucible 12 is shown into which the copper slug 10 is placed, after first disposing at the bottom of the crucible a block 13 of carbon on which lies the anode target 14, in the inclined position which it is to occupy in the completed anode, as shown in Fig. 1.

25 On top of the copper slug 10 is then placed a carbon bushing 15, which serves to hold in place the Kovar element 16, the latter taking the form of a thimble with a lip 17. Within this thimble is placed a weight 18 made of metal having a melting point higher than that of copper, and having a mass adequate to overcome the buoyancy of the Kovar thimble and accordingly acting to sink it into the copper when the latter is in its melted state, as indicated at C in Fig. 3.

30 In operation, when the assembly of Fig. 2 has been placed in the furnace 19 and a suitable degree of heat applied, the copper slug 10 melts and flows down and around the target 14 in known fashion, and the weight 18 draws the thimble 16 down into the molten copper and at 35 the same time draws the lip 17 of the thimble against the top of the carbon bushing until stopped by engagement of the bottom of the bushing with the upper surface of the molten copper, at which time all of the parts occupy the position shown in Fig. 3.

35 The crucible 12 and its associated parts may be removed from the furnace 19, and after allowing the copper to solidify, the partly completed anode will be removed from the crucible, when it 40 presents the appearance shown in Fig. 4, accord-

ing to which it is clear that I have formed a sturdy cast joint between the copper rod 11 and the Kovar seal 16 at the same operation as that of casting the copper, thus eliminating the previously required step of soldering the seal-forming thimble to the copper rod.

After turning off the lip 17 of the thimble 16, the carbon bushing 15 may be slid off the Kovar thimble and can be used as many times as its condition permits, together with the carbon block 13 and the crucible 12, these being permanent parts of my novel apparatus. The anode is now ready to be machined in known fashion, the top edge of the thimble 16 being preferably tapered, as indicated at 21 in Fig. 1, where it enters the glass press press 22 to form the Kovar seal in known manner. The anode illustrated in Fig. 1 is a complete article of manufacture, ready for its intended use in an X-ray tube, and is a unit capable of being stored with other like units, transported as such, and installed at will.

I claim:

1. An anode unit for an X-ray tube comprising a copper supporting rod, a cylindrical Kovar metal seal element having one of its peripheral edges 25

cast in said copper supporting rod to embed the outer surface thereof an appreciable distance in said copper rod, and the opposite end of said cylindrical seal element being embedded in the glass press for said tube.

2. A complete anode unit for an X-ray tube, comprising a copper supporting rod having cast in one end thereof a Kovar metal seal elements in the form of a thimble, the closed end of said thimble being cast in the copper rod to form a molecular union therebetween, and the open end of said thimble being embedded in the glass press for said tube.

3. A complete anode unit for an X-ray tube, comprising a copper supporting rod having cast in one end thereof a Kovar metal seal element in the form of a thimble, the closed end of said thimble being cast in the copper rod to form a molecular union therebetween, and the open end of said thimble being embedded in the glass press for said tube, the other end of said copper rod being bevelled and having cast therein a refractory metal target.

NELSON H. STEWART.